



US005286265A

**United States Patent [19]**

A'Court et al.

[11] Patent Number: 5,286,265

[45] Date of Patent: Feb. 15, 1994

## [54] CARBAMATES, THEIR PRODUCTION AND USE AS FUELS ADDITIVES

[57]

## ABSTRACT

[75] Inventors: **Richard A'Court, Beverley; William J. Fox, London; John E. Hamlin; Sean P. O'Connor, both of Hull, all of United Kingdom**

The invention relates to an internal combustion fuel concentrate comprising: (a) from 1 to 95% of a chlorine-free carbamate prepared by reacting a carbamate of formula

[73] Assignee: **BP Chemicals Limited, London, England**

[21] Appl. No.: 868,485

[22] Filed: Apr. 14, 1992

#### Related U.S. Application Data

[62] Division of Ser. No. 737,457, Jul. 29, 1991, Pat. No. 5,126,477, which is a division of Ser. No. 305,724, Jul. 31, 1989, Pat. No. 5,103,041.

**[30] Foreign Application Priority Data**

Jun. 25, 1987 [GB] United Kingdom ..... 8714872  
Jun. 25, 1987 [GB] United Kingdom ..... 8714873  
Jun. 25, 1987 [GB] United Kingdom ..... 8714874

[51] Int. Cl.<sup>5</sup> ..... C10L 1/22  
[52] U.S. Cl. ..... 44/387; 44/419;

[58] Field of Search 44/329 44/387 329 410

[56] References Cited

## U.S. PATENT DOCUMENTS

|           |         |                     |        |
|-----------|---------|---------------------|--------|
| 4,236,020 | 11/1980 | Lewis et al. ....   | 44/387 |
| 4,274,837 | 6/1981  | Lilburn .....       | 44/387 |
| 5,103,041 | 4/1992  | A'Court et al. .... | 44/387 |
| 5,126,477 | 6/1992  | A'Court et al. .... | 44/387 |
| 5,167,670 | 12/1992 | Johnson .....       | 44/387 |

*Primary Examiner—Jacqueline V. Howard  
Attorney, Agent, or Firm—Brooks Haidt Haffner &  
Delahunty*



with a compound of the formula  $R - OH$  (VI) in the presence of either a strong organic base or a tetra hydrocarbyl titanate so as to exchange the group  $R$  in formula (I) with a group  $R^1$  in formula (II), and (b) a fuel compatible solvent therefor. In the formula (I)  $R$  is a hydrocarbyl or substituted hydrocarbyl group and  $R^1$  is a hydrocarbyl or a hetero-substituted hydrocarbyl group different from  $R$ . In formula (I),  $X$  and  $Y$  are independently any of hydrogen, a hydrocarbyl group, or the group of the formula



where Z is either a divalent hydrocarbyl, a substituted hydrocarbyl group or the group of formula



in which  $n=0$  to 4 and  $m=1$  to 4, and R is hydrocarbyl a substituted hydrocarbyl, provided that if either one of X or Y is the group of formula (II), the other of X or Y is hydrogen.

**15 Claims, No Drawings**

**CARBAMATES, THEIR PRODUCTION AND USE  
AS FUELS ADDITIVES**

This application is a division of application Ser. No. 5 07/737,457 filed Jul. 29, 1991 now U.S. Pat. No. 5,126,477 which in turn is a division of application Ser. No. 07/305,724 filed on Jan. 31, 1989 now U.S. Pat. No. 5,103,041.

The present invention relates to novel carbamates, 10 their production and their use as fuels additives.

Carbamates are useful in agrochemicals, resins, plasticizers and monomers. A number of therapeutic applications include use as antipyretics, diuretics and antiseptics. A widely used method for the production of carbamates is the reaction of an alkyl isocyanate with an alcohol. A disadvantage of this method is that alkyl isocyanates are highly toxic materials. Other reported methods for producing carbamates are disclosed in Japan Kokai 77, 14745 wherein NaOMe/MeOH, PhNH<sub>2</sub> and (MeO)<sub>2</sub> CO are reacted to produce PhNHCO<sub>2</sub>Me, Japan Kokai 79, 163528 which discloses a similar reaction using NaOMe, piperidine, imidazole, carbonyldimidazole, N-methylpyrrolidone or morpholine, U.S. Pat. No. 4,258,683 wherein aromatic amines are reacted with organic carbonates in the presence of zinc and stannous salts, and U.S. Pat. No. 4,268,684 wherein there is disclosed a similar reaction to that of U.S. Pat. No. 4,268,683 except that cabaltous salts are used instead of zinc and stannous salts. 30

Carbamates have also been used as additives to fuels.

A specific problem thought to involve deposit formation in the combustion chamber is that of octane requirement increase (generally abbreviated to ORI). The problem of ORI is addressed by U.S. Pat. No. 4,236,020, the solution to the problem according to the aforesaid U.S. patent being to add to the fuel a poly(oxyalkylene)-carbamate soluble in a hydrocarbon fuel boiling in the gasoline range. The carbamates of U.S. Pat. No. 40 4,236,020 comprise a hydrocarboxy-terminated poly(oxyalkylene) chain or at least 5 oxyalkylene units containing 2 to 5 carbon atoms per oxyalkylene unit bonded through an oxycarbonyl group to a nitrogen atom of ethylenediamine. Preferred carbamates are those described by the general formula:



in which g is an integer 2 to 5, j is an integer such that the molecular weight of the compound is in the range of about 1,200 to about 5,000, Z is a hydrocarbyl of 1 to 30 carbon atoms and sufficient of the oxyalkylene units in the compounds are other than ethylene to render the compounds soluble in hydrocarbon fuels boiling in the gasoline range. The only method disclosed for preparing the carbamates is the reaction of a suitable capped polyether alcohol with phosgene to form a chloroformate followed by reaction of the chloroformate with ethylene diamine to form the active carbamate. A problem associated with this route to carbamates is the use of phosgene which not only is highly toxic but also can lead to products contaminated with chlorine.

We have now found an improved process for the production of carbamates wherein strong organic bases are used as the catalyst.

Accordingly, in a first aspect, the present invention provides a process for the production of a carbamate having the formula:



wherein X and Y are independently either hydrogen, a hydrocarbyl group or a hetero-substituted hydrocarbyl group or the group of formula



wherein Z is either a divalent hydrocarbyl or substituted hydrocarbyl group or a group of the formula:



in which n=0 to 4 and m=1 to 4, and R is a hydrocarbyl or substituted hydrocarbyl group, provided that if either one of X or Y is the group of formula (II), the other of X or Y is hydrogen, which process comprises reacting either a compound of the formula:



35 wherein X and Y are independently either hydrogen, a hydrocarbyl group, or a hetero-substituted hydrocarbyl group, with a dihydrocarbyl carbonate having the formula:



wherein independently R is as defined above in the presence as catalyst of a strong organic base and in the proportions necessary to produce either a mono-carbamate or a bis-carbamate.

Preferably at least one mole of the compound of formula (IV) per mole of the dihydrocarbyl carbonate 50 of formula (V) is employed.

The compound of formula (IV) may be either ammonia (X=Y=H), a primary amine (either of X or Y=H) or a secondary amine (neither of X or Y=H). The amine may suitably be either a monoamine or a polyamine. X and Y may be independently either a hydrocarbyl group of a hetero-substituted hydrocarbyl group. Suitably the hydrocarbyl group may be an aliphatic hydrocarbyl group, of which alkyl groups are preferred. Examples of suitable hydrocarbyl groups include methyl, ethyl, propyl or butyl groups. Alternatively, X and Y may be independently a hetero-substituted hydrocarbyl group. Suitably, the hetero-substituted hydrocarbyl group may be an aliphatic hydrocarbyl group substituted by nitrogen or oxygen, preferably a group of the formula —P—Q, wherein P is an alkylene or polyalkylene group, for example a C<sub>1</sub> to C<sub>4</sub> alkylene group or a poly-C<sub>1</sub> to C<sub>4</sub> alkylene group, and Q is either an NH<sub>2</sub>, —OH or a heterocyclic group, for

60

65

example morpholine or piperazine, or a substituted heterocyclic group, for example piperazine. Examples of suitable compounds (IV) wherein X and Y are independently hetero-substituted hydrocarbyl groups include alkanolamines, for example ethanolamine, and compounds of formula (IV) wherein:

X = H and Y = CH<sub>2</sub>CH<sub>2</sub>NH<sub>2</sub>

(i)

X = H and Y = CH<sub>2</sub>CH<sub>2</sub>CH<sub>2</sub>N      O, and

(ii) 10

X = H and Y = CH<sub>2</sub>CH<sub>2</sub>CH<sub>2</sub>N      NH.

(iii) 15

Finally, the compound (IV) in which X and Y are independently hetero-substituted hydrocarbyl groups, may be an alkylene polyamine or a polyalkylene polyamine, suitably wherein the alkylene group is a C<sub>1</sub>–C<sub>4</sub> alkylene group, for example ethylene diamine, diethylene triamine, triethylene tetramine, and the like.

In the dihydrocarbyl carbonate of formula (V) the groups R are independently hydrocarbyl group which may suitably be alkyl groups, preferably C<sub>1</sub> to C<sub>4</sub> alkyl groups, more preferably methyl groups. Alternatively, the dihydrocarbyl carbonate of formula (V) may be a cyclic carbonate, for example ethylene carbonate or propylene carbonate.

The process may be operated in the presence or absence of an added solvent. Suitable solvents include liquid hydrocarbon solvents, for example the mixed aromatic solvent designated A260 commercially available from BP Chemicals Limited.

The catalyst is a strong organic base. A preferred strong organic base is an amidine. By the term amidine is meant a compound containing the grouping:



wherein the free valencies on the nitrogen atoms are attached to either carbon atoms or hydrogen and the free valency on the carbon atom is attached to either another carbon atom or nitrogen. In the case that the free valency on the nitrogen is attached to nitrogen the amidine is a guanidine.

A preferred class of amidine is the cyclic amidines. Cyclic amidines are defined as those amidines wherein at least one of the nitrogen atoms is part of an alicyclic or heterocyclic substituted or unsubstituted hydrocarbyl ring. In the case where the amidine is a guanidine then any two or the three nitrogen atoms may be in the same or different rings. Those nitrogen atoms which are not part of any said ring may form part of a substituted or unsubstituted hydrocarbyl group.

A preferred class of cyclic amidine is that in which the amidine group can form part of a fused ring system containing 6 and 5 membered rings or 6 and 7 membered rings or two six membered rings, as for example in which has the formula

1,5-diazabicyclo [4.3.0] non-5-ene (DBN)



or

1,8-diazabicyclo [5.4.0] undec-7-ene (DBU) of the formula



or

1,5,7-triazabicyclo [4.4.0] dec-5-ene (TBD) of formula



The amidine may be supported on a suitable support.

25 This may be accomplished by deposition of the amidine on a support or by chemical bonding of the amidine to a suitable support. Suitable supported amidine catalysts are described in, for example, our EP-A-0168167.

30 As an alternative to an amidine, the strong base may comprise a Lewis base and an epoxide. The term Lewis base is generally understood to mean a compound containing an unshared pair of electrons capable of sharing with an acid. The terms Lewis base and amidine are not therefore mutually exclusive. The Lewis base may suitably be an organic compound containing triivalent nitrogen or phosphorus, for example an amine or a phosphine. The epoxide may suitably be a substituted or unsubstituted C<sub>2</sub> to C<sub>8</sub> alkylene oxide, preferably either ethylene oxide, propylene oxide or butylene oxide.

35 40 As regards the reaction conditions, the process may suitably be operated at a temperature in the range from 0° to 100° C., more preferably from 15° to 75° C., most preferably from 20° to 25° C., and the pressure may be either atmospheric or superatmospheric, for example from 1 to 10 bar.

45 The process may be operated batchwise or continuously, preferably continuously.

An advantage of using the process of the present invention for the production of carbamates is that it avoids the use of phosgene and its associated disadvantages.

The group R in the carbamate of formula (I) can be exchanged for a group R<sup>1</sup> by a process which comprises reacting the carbamate of formula (I) with a compound of the formula:



50 55 60 wherein R<sup>1</sup> is a hydrocarbyl or hetero-substituted hydrocarbyl group different from R, in the presence as catalyst of either a strong organic base or a tetrahydrocarbyl titanate.

65 The group R<sup>1</sup> in the compound of formula (VI) may suitably be any of the groups R as defined for the carbamate of formula (I), provided it is not identical to the group R. Hydrocarbyl groups substituted with nitrogen and/or oxygen, for example hydrocarbyl polyether groups, may be used.

In a preferred embodiment of the present invention there is provided a process for the production of a carbamate suitable for use as a detergent additive to internal combustion engine fuels wherein the group R<sup>1</sup> in the compound of formula (VI) is a hydrocarbyl or hetero-substituted hydrocarbyl group of a molecular weight and composition such as to impart fuel solubility.

A preferred compound of formula (VI) for this purpose is a polyalkylene glycol (PAG) formed by the reaction of a hydroxylic compound, which may be either an alcohol, or a phenol with an alkylene oxide, and may suitably have a molecular weight in the range from about 500 to 10,000, preferably from 1200 to 5000. PAGs are more fully described in the aforesaid U.S. Pat. No. 4,236,020, the disclosure of which in respect of suitable PAGs is incorporated by reference herein. The PAG should contain sufficient oxyalkylene units other than ethyleneoxy to effect solubility in internal combustion engine fuels. A particularly suitable compound of formula (VI) for use in the process of the invention is a polyoxyalkylene glycol obtained by the reaction of p-dodecylphenol with butylene oxide and having a molecular weight of about 2,000, which material is commercially available as BREOX (RTM) PC 1362 from Hythe Chemicals Limited. Another preferred class of compound of formula (VI) suitable for use in the production of detergent additives is polyalkylene glycols produced by the hydroxyalkylation, suitably by reaction with alkylene oxides, or amines, for example 30 ethylene diamine or aminopropylmorpholine.

As catalyst for the exchange reaction there is used either a strong organic base or a tetrahydrocarbyltitanate. Suitable strong organic bases are those as hereinbefore described in relation to the preparation of carbamates of the formula (I). The same strong organic base or a different strong organic base, preferably the same, may be used in the exchange reaction as in the preparation of the carbamate of formula (I). Suitably the tetrahydrocarbyltitanate may be a tetraalkyltitanate. Suitably the alkyl group of the tetraalkyltitanate may be a C<sub>1</sub> to C<sub>4</sub> alkyl group. An example of a suitable tetraalkyltitanate is tetraisopropyltitanate.

It is preferred to react the compound of formula (I) with the compound of formula (VI) in the presence of a suitable solvent. Suitably the solvent may be a hydrocarbon solvent, for example the mixed aromatic hydrocarbon solvent identified as A260 which is commercially available from BP Chemicals Limited.

As regards the reaction conditions for reacting the compound of formula (I) with the compound of formula (VI), the temperature may suitably be elevated, preferably in the range from 100° to 300° C., and the pressure may be either atmospheric or superatmospheric.

A particular advantage of the process claimed for the production of detergent additives is that it provides a chlorine-free product, in contrast to prior art processes, such as that of U.S. Pat. No. 4,236,020.

In another aspect the present invention provides an internal combustion engine fuel concentrate composition comprising as a first component from 1 to 95% by weight of a carbamate of the formula (I) wherein the group R is a hydrocarbyl or substituted hydrocarbyl group of a molecular weight and composition such as to 65 impart fuel solubility as produced by a process as hereinbefore described and as a second component a fuel compatible solvent therefor.

The fuel compatible solvent for the compound of the formula (II) may suitably be an internal combustion engine fuel.

Preferably the carbamate is a mono-carbamate.

In another aspect the invention comprises an internal combustion engine fuel composition comprising a major proportion of an internal combustion engine fuel and a minor proportion of the concentrate composition as hereinbefore described.

The amount of the concentrate composition present in the fuel composition may suitably be such as to provide a concentration of the compound of formula (I) in the fuel composition in the range from 10 to 10,000 p.p.m. by weight.

The internal combustion engine fuel is preferably a fuel boiling in the gasoline range. The fuel composition may incorporate additives conventionally employed in fuels compositions. Such additives may be incorporated either into the fuel concentrate or directly into the fuel composition.

In another aspect the present invention provides as novel compounds carbamates of the formula (I) other than those disclosed in U.S. Pat. No. 4,236,020 and in particular those wherein X and Y are independently the group of formula —P—Q as hereinbefore described and their reaction products with a compound of formula (VI), suitably wherein R<sup>1</sup> is a hydrocarbyl or hetero-substituted hydrocarbyl group of a molecular weight and composition such as to impart fuel solubility.

The invention will now be further illustrated by reference to the following Examples.

#### PREPARATION OF MONOCARBAMATE OF THE FORMULA (I)

##### EXAMPLE 1

Dimethylcarbonate (9.0 g) and n-butylamine (7.3 g) were mixed with TBD (0.05 g) and allowed to stand at room temperature. After 6 h a sample of the liquid product was shown, by gc/ms, to be methyl N-(n-butyl) carbamate (95% yield).

##### EXAMPLE 2

Dimethylcarbonate (9.0 g) and n-propylamine (5.9 g) were mixed with TBD (0.05 g) according to Example 1. The product was shown by gc/ms to be methyl N-(n-propyl) carbamate (93% yield).

##### EXAMPLE 3

Dimethylcarbonate (9.0 g) and ethanolamine (4.7 g) were mixed with TBD (0.05 g) according to Example 1. The product was shown by gc/ms to be methyl N-(2-hydroxyethyl) carbamate (86% yield).

##### EXAMPLE 4

Example 1 was repeated replacing the dimethylcarbonate with diethylcarbonate (9.2 g). The liquid product was shown by gc/ms to be ethyl N-(n-butyl) carbamate (92% yield).

##### Comparison Test 1

Example 1 was repeated in the absence of TBD. Only starting material was recovered.

##### Comparison Test 2

Example 1 was repeated replacing the TBD with triethylamine (0.05 g). The liquid product was shown

by gc/ms to be methyl N-(n-butyl) carbamate (6% yield).

## EXAMPLE 5

Example 1 was repeated replacing TBD with DBU. 5  
The liquid product was shown by gc/ms to be methyl N-(n-butyl) carbamate (65% yield).

## EXAMPLE 6

Example 1 was repeated replacing TBD with DBN. 10  
The liquid product was shown by gc/ms to be methyl N-(n-butyl) carbamate (30% yield).

## EXAMPLE 7

A mixture of ethanolamine (50.6 g), dimethylcarbonate (74.8 g), TBD (1.0 g) and m-xylene (10 ml) was 15 refluxed for 3 hours (ca. 80° C.). The mixture was evaporated under reduced pressure giving the product as a clear liquid (84 g). NMR analysis indicated the product to be methyl [N-(2-hydroxyethyl)] carbamate. 20

## EXAMPLE 8

A mixture of N-(2-aminoethyl) piperazine (28 g), dimethylcarbonate (20 g) and TBD (1.0 g) was left to stand open to the atmosphere for 120 hours. The mixture was evaporated under reduced pressure giving the product (38.75 g) identified by NMR to be methyl N-[2-(N<sup>1</sup>-piperazinol)ethyl] carbamate. 25

## EXAMPLE 9

A mixture of N-(3-aminopropyl) pipecoline (37.1 g), dimethylcarbonate (23.0 g) and TBD (1.0 g) was allowed to stand open to the atmosphere for 120 hours. The mixture was evaporated under reduced pressure giving the product (46.1 g), identified by NMR to be methyl N-[3-(N<sup>1</sup>-pipercolino)propyl] carbamate. 35

## EXAMPLE 10

—X=H,



in formula (I).

## Step (A)

A mixture of N-(3-aminopropyl) morpholine (57.1 g), dimethyl carbonate (42 g) and TBD (1.0 g) was refluxed for 6 hours with a nitrogen sparge. The resultant mixture was evaporated under reduced pressure to give the product as a clear yellow liquid (74 g). NMR analysis indicated the product to be methyl N-[3-(N<sup>1</sup>-morpholino)propyl] carbamate. 50

## Step (B)

The intermediate carbamate from Step A (16.5 g), 60 BREOX PC 1362 (114 g) and TBD (1.0 g) were stirred at 150° C. for 3.5 hours with a nitrogen sparge. The mixture was cooled, treated with toluene (50 ml) and magnesium sulphate (1.0 g) and allowed to stand. The mixture was then filtered and evaporated under reduced pressure to give the product as a clear pale yellow liquid. 65

Analysis: % Nitrogen found = 1.46

## EXAMPLE 11

—X=H,



in the formula (I).

## Step (A)

A mixture of N-(2-aminoethyl)piperazine (20 g), dimethylcarbonate (33.6 g) and DBU (0.2 g) was stirred at 80°-120° C. for 2 hours with a nitrogen sparge. The mixture was cooled and filtered to give the product as a clear orange-yellow liquid. NMR analysis indicated the product to be methyl N-[2-(N<sup>1</sup>-piperazino)ethyl] carbamate. 15

## Step (B)

the intermediate carbamate product from Step A (10.8 g, containing DBU catalyst carried through from Step A) and BREOX PC 1362 (136 g) were stirred at 120°-140° C. for 3 hours with a nitrogen sparge. The product was cooled and filtered to give a clear yellow liquid. 20

Analysis: % Nitrogen = 1.10.

## EXAMPLE 12

A mixture of methyl N-[3-(N<sup>1</sup>-morpholino)propyl] carbamate (the intermediate product obtained from Example 10, Step A) (10 g), 1-octanol (15.0 g), m-xylene (25 ml) and TBD (0.2 g) was refluxed for 1 hour. The mixture was evaporated under reduced pressure giving the product as a light yellow liquid (30.4 g). NMR analysis indicated the product to be n-octyl N-[3-(N<sup>1</sup>-morpholino)propyl] carbamate. 30

## EXAMPLE 13

A mixture of methyl N-[3-(N<sup>1</sup>-morpholino)propyl] carbamate (the intermediate product obtained from Example 10, Step A) (5.2 g), polyalkylene glycol (PAG 45 B225 from Hythe Chemicals Limited) (49.5 g), TBD (0.4 g) and m-xylene (33.4 g) was stirred at 140° C. with a nitrogen sparge for 2 hours. The mixture was evaporated under reduced pressure giving the product as a viscous yellow liquid (45 g). 40

## EXAMPLE 14

A mixture of methyl N-[2-(N<sup>1</sup>-piperazino)ethyl] carbamate (the product of Example 8) (5.8 g), 1-octanol (4.3 g) and TBD (0.6 g) was heated at 150° C. for 2 hours. The mixture was evaporated under reduced pressure giving a red-brown product (8.2 g), indicated by NMR analysis to be n-octyl N-[2-(N<sup>1</sup>-piperazino)ethyl] carbamate. 50

## EXAMPLE 15

A mixture of methyl N-[3-(N<sup>1</sup>-morpholino)propyl] carbamate (the intermediate product obtained from Example 10, Step A) (16.0 g), BREOX PC 1470 [(ex Hythe Chemicals Limited, prepared by reaction of p-dodecylphenol (1 mole) with butylene oxide (15 moles)] (10.35 g) and TBD (0.9 g) was stirred at 150° C. with a nitrogen sparge from 4.25 hours. The mixture was then cooled and treated with toluene (50 ml) and magnesium 60



wherein R<sup>1</sup> is a hydrocarbyl or a hetero-substituted hydrocarbyl group different from R in the presence of either a strong organic base or a tetrahydrocarbyl titanate so as to exchange the group R in formula (I) with a group R<sup>1</sup>, and as a second component a fuel compatible solvent therefor.

2. A concentrate composition according to claim 1 wherein the solvent is an internal combustion engine fuel.

3. A concentrate composition according to claim 1 wherein the carbamate of formula (I) is mono-carbamate.

4. An internal combustion engine fuel composition comprising a major proportion of an internal combustion engine fuel and a minor proportion of the concentrate composition as claimed in claim 1.

5. A composition according to claim 4 wherein the amount of the concentrate composition is such as to 20 provide a concentration of the compound of formula (I) in the final composition in the range from 10 to 10,000 p.p.m. by weight.

6. A composition according to claim 5 wherein the internal combustion engine fuel is a fuel boiling in the gasoline range.

7. A concentrate composition according to claim 1 wherein the carbamate of formula I is a biscarbamate.

8. A concentrate composition according to claim 3 30 wherein said monocarbamate is methyl N-[3-(N<sup>1</sup>-morpholino) propyl] carbamate.

9. A concentrate composition according to claim 3 wherein said monocarbamate is N-[2-(N<sup>1</sup>-piperazino) 35 ethyl] carbamate.

10. A concentrate composition according to claim 3 wherein the monocarbamate is methyl N-(n-butyl) carbamate.

11. A concentrate composition according to claim 3 5 wherein the monocarbamate is methyl N-(n-propyl) carbamate.

12. A concentrate composition according to claim 3 wherein the monocarbamate is methyl N-(2-hydroxyethyl) carbamate.

13. A concentrate composition according to claim 3 10 wherein the monocarbamate is ethyl N-(n-butyl) carbamate.

14. A concentrate composition according to claim 3 15 wherein the monocarbamate is N-[3-(N<sup>1</sup>-piperolino) propyl] carbamate.

15. A lubricating oil concentrate according to claim 1 wherein the carbamate of formula (I) is prepared by reacting a compound of formula IV



25 with a dihydrocarbonyl carbamate having the formula V:



at a temperature in the range of from 0° to 100° C. and a pressure in the range from 1 to 10 bar, the designation X, Y and R having the meanings attributed to them in claim 1.

\* \* \* \* \*

UNITED STATES PATENT AND TRADEMARK OFFICE  
CERTIFICATE OF CORRECTION

PATENT NO. : 5,286,265

Page 1 of 2

DATED : February 15, 1994

INVENTOR(S) : Richard A'Court, William J. Fox, John E. Hamlin and  
Sean P. O'Connor

It is certified that error appears in the above-identified patent and that said Letters Patent is hereby corrected as shown below:

In the Abstract, 5th from last line, close the parenthesis after  
"H" so that it reads --(NH) --  
n

Col. 1, l. 25, correct the spelling of the word  
"carbonyldiimidazole"

Col. 1, l. 42, change "or" to --of--

Col. 1, l. 54, correct the spelling of the word "hydrocarbyl"

Col. 2, l. 12, there should be a colon (:) after the word  
"formula:"

Col. 2, l. 21, close the parenthesis after "H"

Col. 3, l. 68, strike "in which has the formula"

Col. 4, line 1, after "(DBN)" insert --which has the formula--

Col. 4, l. 35, correct the spelling of the word "trivalent"

Col. 5, l. 62, correct the spelling of the word "first"

Col. 6, l. 11, after "as" strike "a"

Col. 8, l. 23, correct the spelling of the word "carbamate"

Col. 8, l. 67, after "sparge" change "from" to --for--

Col. 9, l. 59, should read "The nitrogen"

UNITED STATES PATENT AND TRADEMARK OFFICE  
CERTIFICATE OF CORRECTION

PATENT NO. : 5,286,265

Page 2 of 2

DATED : February 15, 1994

INVENTOR(S) : Richard A'Court, William J. Fox, John E. Hamlin and  
Sean P. O'Connor

It is certified that error appears in the above-identified patent and that said Letters Patent is hereby  
corrected as shown below:

Claim 1, col. 10, line 59, formula (III) should read --alkylene)<sub>m</sub>(NH<sub>n</sub>  
(alkylene)<sub>m</sub>--

Signed and Sealed this

Sixteenth Day of August, 1994

Attest:



BRUCE LEHMAN

Attesting Officer

Commissioner of Patents and Trademarks